

Patented May 6, 1924.

1,493,205

# UNITED STATES PATENT OFFICE.

ISIDORE JASCOWITZ AND JOHN ROSENBAUM, OF LONDON, ENGLAND, ASSIGNORS TO  
R. J. CORPORATION, LIMITED, OF LONDON, ENGLAND.

## CLEANING OF METALS BY ELECTROLYSIS.

No Drawing.

Application filed May 4, 1921. Serial No. 466,710.

To all whom it may concern:

Be it known that we, ISIDORE JASCOWITZ and JOHN ROSENBAUM, subjects of the King of Great Britain, residing at 66 Greenfield 5 Street, London, E., England, have invented a new and useful Cleaning of Metals by Electrolysis (for which we have filed application in Great Britain August 22, 1918, No. 13,642); and we do hereby declare that the 10 following is a full, clear, and exact description of the invention, which will enable others skilled in the art to which it appertains to make and use the same.

This invention relates to a novel process 15 for the electrolytic cleaning of metal articles.

It has been proposed to remove scale and oxide from metal plates, wires, strip or ribbon by passing the said plates or the like 20 through an electrolytic solution consisting of a weak solution of sulphuric or hydrochloric acid or caustic soda.

Now this invention consists in the utilization 25 of an improved electrolyte in which the metal articles to be cleaned are suspended or placed in an electrolytic-vat, in electrical connection with the cathode, the anodes being suitably made of iron. The electrolyte consists of spent caustic melt solution, obtained 30 in the fusion process in the manufacture of a variety of chemicals such as B-naphthol, phenol, alizarine, resorcin, and is a compound of caustic soda and sulphite, sulphate and carbonate of sodium, together 35 with organic residues. As a typical melt may be taken a residue obtained in the manufacture of phenol and which would have a composition approximately as follows:—

By weight.

|                     |         |
|---------------------|---------|
| Caustic soda        | 50%     |
| Sodium sulphite     | 28%     |
| Sodium sulphate     | 8%      |
| Sodium carbonate    | 8%      |
| Phenol (traces) say | 1 to 2% |

Or, in lieu thereof a prepared solution having 45 the composition or practically the composition, of the caustic melt solution, as for example, caustic soda solution admixed with inorganic salts, such as sodium sulphate, sodium sulphide and sodium sulphite, and with organic compounds, such as phenolates and salicylates, which serve to conduct the electric current through the electrolyte. The 50 electrolyte should have a strength of 15 to

20 per cent and is, in practice advantageous-ly heated to a temperature of about 90° C.

By the process it is found possible to remove from iron, steel and other metal articles, all oils, fats, greases, paints, rust and scale with which their surfaces have become coated and to produce thoroughly clean surfaces, thus obtaining in a single process or operation a result which has heretofore only been obtainable by subjecting the articles to 60 be cleaned to two distinct operations. The process, therefore, effects an economy in 65 time and labour.

### Claims:

1. The herein described process for the 70 electrolytic cleaning of iron, steel and other metals, which consists in subjecting the article to be cleaned to electrolytic action in an electrolyte containing a large proportion by weight of caustic soda, a smaller proportion 75 by weight of sodium sulphite, and smaller proportions by weight of sodium sulphate and sodium carbonate.

2. The herein described process for the 80 electrolytic cleaning of iron, steel and other metals, which consists in subjecting the article to be cleaned to electrolytic action in an electrolyte containing a large proportion by weight of caustic soda, a smaller proportion by weight of sodium sulphite, and smaller 85 proportions by weight of sodium sulphate and sodium carbonate, and smaller quantities of phenolate and salicylate of soda.

3. The herein described process for the 90 electrolytic cleaning of iron, steel and other metals, which consists in subjecting the article to be cleaned to electrolytic action in an electrolyte containing approximately 50% by weight of caustic soda, 28% by weight of sodium sulphite, and 8% by weight each of 95 sodium sulphate and sodium carbonate.

4. The herein described process for the 100 electrolytic cleaning of iron, steel and other metals, which consists in subjecting the article to be cleaned to electrolytic action in an electrolyte containing approximately 50% by weight of caustic soda, 28% by weight of sodium sulphite, and 8% by weight each of sodium sulphate and sodium carbonate, and 1.5% by weight of phenolate of soda. 105

5. The herein described process for the 110 electrolytic cleaning of iron, steel and other metals, which consists in subjecting the article to be cleaned to electrolytic action in an electrolyte containing approximately 50% 110

by weight of caustic soda, 28% by weight of sodium sulphite, and 8% by weight each of sodium sulphate and sodium carbonate, and 1.5% by weight of salicylate of soda.

- 5 6. The herein described process for the electrolytic cleaning of iron, steel and other metals, which consists in subjecting the article to be cleaned to electrolytic action in an electrolyte consisting of a spent caustic melt  
10 solution obtained in the fusion process in the

manufacture of chemicals such as B-naphthol, phenol, alizarine and resorcin, and containing a large proportion by weight of caustic soda, a smaller proportion by weight of sodium sulphide, smaller proportions by weight each of sodium sulphate and sodium carbonate. 15

ISIDORE JASCOWITZ.  
JOHN ROSENBAUM.